

## UNITED STATES PATENT OFFICE

2,562,065

## CARBURIZING SALT BATH

Edna L. Sawyer, Stamford, and Northrup W. Marr, Springdale, Conn., assignors to American Cyanamid Company, New York, N. Y., a corporation of Maine

No Drawing. Application November 29, 1950,  
Serial No. 198,226

3 Claims. (Cl. 148—27)

1

The present invention relates to salt mixtures which, when in a molten condition at elevated temperatures, are adapted for carburizing ferrous metal, a bath made from such salt mixtures, and a process of using the bath.

It is an object of this invention to provide a case carburizing bath that will give effective case depths of at least 16 mils in one hour at 1600° F. consistently, but which, at the same time, will not leave an insoluble sludge on the article after it is removed from the bath, oil quenched, and shaken in hot water. It is a further object of the present invention to provide an easy washing carburizing bath operable over a temperature range of 1300° to 1750° F. It is a still further object to provide an inexpensive, novel, and effective activator for such a bath, namely, an alkali metal silicate. Still other objects will be obvious from the description of the invention given below.

A cyaniding bath containing unactivated sodium cyanide does not coat the work with insoluble sludges, but is unsuitable as a carburizing bath because it carburizes slowly and gives effective case depths of only about 12 mils at the highest temperature at which it can be operated, namely, around 1550° F., and is further unsatisfactory as a carburizing means since it nitrides the work as well as carburizes it, the case at the surface analyzing about 0.6% C and about 0.5% N.

The usual liquid carburizing bath provides satisfactory case depths through the activation of calcium and barium salts. Such a bath may give an effective case depth of from 16 mils in an hour at 1600° F. to 125 mils in 16 hours at 1750° F. A disadvantage of a bath activated with calcium and barium salts is that these salts sludge, forming oxides and carbonates that adhere to the article when it is withdrawn from the bath and that cannot be dissolved in hot water, but must be removed from the article by chemical and/or mechanical means.

An easy washing carburizing bath has now been found that incorporates the easy washing characteristics of a cyaniding bath with the high carburizing activity of a calcium salt-activated bath. The bath of the present invention, unlike a cyaniding bath, is operable up to 1750° F. and gives satisfactory case depths even though it contains no alkaline earth activator. The bath of the present invention is further characterized by its high activity in commercial-size pots, its ease of maintaining a good cover, low sodium cyanide loss, and low nitriding.

The present invention involves a completely new concept in carburizing baths. In the past, it has been the understanding of practitioners using soluble carburizing baths, that the presence of a considerable amount of alkaline material tended to stabilize the carburizing activity of the bath, reducing carbon penetration to a constant

2

and unacceptable level. For example, while the highly alkaline bath might give case depths of 16 mils in the beginning of its operation, penetration would soon drop to the order of 12–14 mils or less. It was believed that this reduced inactivity was caused by stabilization of the bath by the alkaline materials present. A standard method of correcting excess alkalinity has been to add acid materials to the bath. Examples of such acid materials are free silica and the sodium acid silicates. Thus corrected, the bath retained its reactivity and gave good carburizing penetration over a long period of time.

The present invention demonstrates that a highly alkaline bath can be prepared containing substantial quantities of alkali metal containing no acidic groups, and that the bath gives consistent high penetration over a long period of time. This combination of high alkalinity and alkali metal silicates containing no acidic elements is unobvious and, so far as the inventors are aware, there is no suggestion of the combination in the prior art. In the following description, wherever alkali metal silicates are mentioned, it is to be understood they are the normal salts, containing no acidic hydrogen. They may be added as such or formed in situ in the bath.

The bath contemplated in the present invention gives effective case depths on fracture up to about 32 mils during a four-hour treatment at 1600° F. in the bath, and the film of adherent salts after an oil quench is so soluble that it may be removed simply by shaking the work in hot water a few times. Adherent salts from holes  $\frac{1}{8}$  inch in diameter and  $\frac{1}{2}$  inch deep are easily removed by such means.

When making up the bath, a salt mixture with the following range of ingredients may be used (parts by weight):

|    |                                                                                 |     |      |
|----|---------------------------------------------------------------------------------|-----|------|
| 40 | Sodium chloride                                                                 | 20  | —50  |
|    | Sodium carbonate                                                                | 25  | —45  |
|    | Sodium cyanide                                                                  | 15  | —35  |
| 45 | Anhydrous sodium silicate, sufficient to provide an SiO <sub>2</sub> content of | 0.5 | —5.5 |
|    | Graphite                                                                        | 0.3 | —1.0 |

Various equivalents may be used for the above substances. For example, various other water-soluble cyanogen-forming compounds may be used instead of sodium cyanide, namely, other alkali metal cyanides, cyanates, cyanamides, and the like. Organic cyanogen compounds are also suitable as, for example, cyanamide, dicyanamide, melamine, melam, melem, melon, ammeline, ammeliide, hydrogen cyanide polymers, and the like. The sodium carbonate of the bath may be substituted for, in total or in part, by other alkali metal carbonates, and the sodium chloride may be similarly substituted by other alkali metal chlorides. The sodium silicate used

may vary widely in its  $\text{Na}_2\text{O}:\text{SiO}_2$  ratio and may be replaced by potassium silicate. However, a sodium silicate containing about 50%  $\text{Na}_2\text{O}$  and 50%  $\text{SiO}_2$ , conforming to the approximate molecular formula  $\text{Na}_2\text{SiO}_3$ , is preferred.

Although the quantity ranges listed above are operable and are contemplated by the invention, the following composition represents the preferred materials and their preferred ranges (parts by weight):

NaCN, 20-25.  
 $\text{Na}_2\text{SiO}_3$ , 3-10, equivalent to 1.5-5 parts of contained silica.  
 $\text{Na}_2\text{CO}_3$ , 30-35.  
 Graphite, 0.3-1.0.  
 $\text{NaCl}$ , remainder to give 100 parts total.

The 1.5-5.0 parts of silica in the sodium silicate is fairly critical, as a content of less than 0.5 part fails to provide the necessary carbon penetration, while a content of more than 5.5 parts results in excessive sludging in the bath. When using the bath in the silica range of 1.5-4 parts of contained silica (3-8 parts alkali metal silicate) the bath should be replenished daily to maintain a satisfactory carburizing activity.

A significant advantage of the bath of this invention is its ability to give good case depths over a wide range of temperature without developing detrimental working characteristics. In the past it has been customary to use one bath to cover the range 1500°-1650° F. and a second bath to cover the range 1600°-1750° F. It was found that the first bath could not be heated substantially above 1650° F. without foaming or sludging or both, and that the second bath, while having excellent cover and sludge characteristics in the neighborhood of 1700° F. would not give good case depths below 1650° F. In contrast, the bath of the present invention gives excellent case depths with good cover performance and little or no sludging over a range of 1300°-1750° F.

It has further been found that parts carburized in the bath of the present invention have a good clean metallic appearance when washed after an oil quench. It is common knowledge that parts similarly washed after treatment in a barium activated bath are frequently discolored.

Another advantage of the present bath over previous carburizing baths is that it may be operated at a temperature as low as 1400° F., at which temperature it gives a case depth (microscopic) of 8 mils in 4 hours. This possibility permits carburization of intricate work without distortion.

The following example illustrates but does not limit the use of the bath.

#### Example 1

A mixture of salts consisting of 20% sodium cyanide, 30% sodium carbonate, 40% sodium chloride, and 10% sodium silicate (in the form of a commercial alkaline cleaner) with 0.3% graphite was melted and heated to the operating temperature.

As the bath melted, the graphite formed a soft blanket which reduced the loss of cyanide and prevented evaporation of the bath while in use.

To maintain the energizing effect, and to compensate for cyanide loss and drag out from the bath, it is desirable but not absolutely necessary to add to the bath, in the amount of 7-8% of the total bath weight, every working day, a mixture consisting of 10% sodium silicate, 40% sodium cyanide, 50% sodium chloride and 0.3% graphite.

The carburizing performance of this bath on treated work is shown in the following table.

| Treatment No. | Temp.,<br>° F. | Case Depths Obtained on<br>1/4" Dia. SAE 1020 Steel<br>Rods on Fracture, in<br>Mils |    |       |       |
|---------------|----------------|-------------------------------------------------------------------------------------|----|-------|-------|
|               |                | Time, Hours                                                                         |    |       |       |
|               |                | 1                                                                                   | 2  | 3     | 4     |
| 10            |                |                                                                                     |    |       |       |
| 1             | 1,500          | 11                                                                                  | 16 | 20    | 22    |
| 2             | 1,600          | 16                                                                                  | 22 | 28    | 32    |
| 3             | 1,650          | 18                                                                                  | 28 | 32    | 39    |
| 4             | 1,750          | 24                                                                                  | 36 | ----- | ----- |
| 15            |                |                                                                                     |    |       |       |

Essentially, case penetration is equal to that produced using a barium carburizing salt bath.

This is a continuation-in-part of applicants' co-pending Serial No. 89,576, filed April 25, 1949, now abandoned.

The sodium silicate used in the herein examples contained about 50% silica.

#### Example 2

Carburizing comparable to that of Example 1 is obtained with a bath made up from a mixture consisting of 29% sodium cyanide, 39% sodium carbonate, 29% sodium chloride, 3% sodium silicate, and 0.2% graphite replenished daily with a mixture consisting of 40% sodium cyanide, 28% sodium carbonate, 29% sodium chloride, 3% sodium silicate, and 0.2% graphite. The bath so used avoids a slight sludging occasionally encountered in the higher silicate ranges of the bath of Example 1.

While the invention has been described with particular reference to specific embodiment, it is to be understood that it is not to be limited thereto but is to be construed broadly and restricted solely by the scope of the appended claims.

We claim:

1. A mixture adapted upon fusion for the carburizing of ferrous metal articles which consists essentially of alkali metal chloride about 20-50 parts, cyanogen compound about 15-35 parts, anhydrous alkali metal carbonate about 25-45 parts, alkali metal silicate equivalent to about 0.5-5.5 parts of silica, and graphite about 0.1-1.0 part, the parts being by weight.

2. A mixture adapted upon fusion for the carburizing of ferrous metal articles which consists essentially of sodium chloride about 40 parts, sodium cyanide about 20 parts, sodium carbonate about 30 parts, anhydrous sodium silicate equivalent to about 5 parts of silica and graphite about 0.3 part, the parts being by weight.

3. A mixture adapted upon fusion for the carburizing of ferrous metal articles which consists essentially of alkali metal carbonate about 39 parts, anhydrous alkali metal silicate equivalent to about 1.5 parts of silica, alkali metal cyanide about 29 parts, graphite about 0.3 part, and alkali metal chloride to make 100 parts, the parts being by weight.

EDNA L. SAWYER.  
 NORTHRUP W. MARR.

#### REFERENCES CITED

70 The following references are of record in the file of this patent:

#### UNITED STATES PATENTS

Number Name Date  
 76 2,541,085 Morral Feb. 13, 1951